

(No Model.)

E. P. THOMPSON.

MANUFACTURE OF INCANDESCING CARBON FILAMENTS.

No. 401,607.

Patented Apr. 16, 1889.

FIG. 2.



FIG. 1.

ATTEST:

J. M. Murchie  
Carrie E. Davidson

INVENTOR:  
Edward P. Thompson.

By  
Pope, Dugay & Terry

his Attorneys.

# UNITED STATES PATENT OFFICE.

EDWARD P. THOMPSON, OF ELIZABETH, NEW JERSEY.

## MANUFACTURE OF INCANDESCING CARBON FILAMENTS.

SPECIFICATION forming part of Letters Patent No 401,607, dated April 16, 1889.

Application filed March 28, 1887. Serial No. 232,785. (No model.)

*To all whom it may concern:*

Be it known that I, EDWARD P. THOMPSON, a citizen of the United States, residing in Elizabeth, in the county of Union and State of New Jersey, have invented certain new and useful Improvements in Process of Carbonizing Filaments for Incandescent Electric Lamps, of which the following is a specification.

The invention relates to a method of preparing filaments for incandescent electric lamps, in which the fiber is first partially carbonized by being treated by acids and subsequently completely carbonized by heat.

The object of the invention is to provide means for expelling all the oxygen which may be absorbed by the filaments and by the molds carrying them after the filaments are partially carbonized by acids and before they are subjected to heat for completing the carbonization.

The invention consists, in general terms, in first subjecting the filaments to an acid bath after the process described in United States Patent No. 323,372, dated July 28, 1885, in which the filaments are placed in an acidulated saccharine solution—such, for instance, as sulphuric acid containing sugar in solution. After the filaments are removed from this bath they are dried, and being partially carbonized the pores absorb more or less oxygen. It is desired by the present invention to remove such oxygen from the filaments before they are completely carbonized by heat. The filaments are placed upon suitable forms, preferably molds of carbon blocks, before they are placed in a heating-oven. These blocks are more or less porous, and naturally contain a greater or less quantity of oxygen. The present invention involves the expelling of this oxygen also before the molds and the filaments are placed in the carbonizing-oven. For this purpose they are placed in a suitable chamber and immersed in a hydrocarbon liquid, which is then placed under pressure, thereby forcing the liquid into the pores and replacing the oxygen. The molds and filaments are then subjected to the carbonizing process in the usual manner, and as practically all the oxygen has been expelled therefrom the filaments are not injured by being themselves attacked by the oxygen.

The invention will be described in detail in connection with the accompanying drawings, in which Figure 1 illustrates an apparatus for receiving and drying the filaments after they have been partially carbonized by the acid solution. This same apparatus or an equivalent chamber may be employed for treating the filaments with a solution of liquid hydrocarbon for replacing the oxygen. Fig. 2 illustrates the apparatus employed for finally carbonizing the filaments.

Referring to the figures, A represents a suitable chamber, which is preferably air-tight, and in which there are placed molds B, upon which the partially-carbonized filaments are placed. This chamber is provided with a pipe, C, through which steam or hot air is passed for the purpose, in the first instance, of heating the filaments and the molds, thereby drying and stiffening the former before they are carbonized by heat. At a suitable point an outlet, a, provided with a stop-cock, a', leads from the chamber A. The vapors arising from the heating of the chamber may escape through an outlet, a<sup>2</sup>, which at other times may be closed by a valve, a<sup>3</sup>. This device is preferably constructed after the manner of a safety-valve, but is held open during the process of drying and stiffening the filaments.

After the filaments have been heated the chamber is partially filled with a hydrocarbon liquid through the opening a or in any other convenient manner, and heat is again applied through the pipe C. The heat serves to vaporize a portion of the hydrocarbon, and, the valve a' being closed, a greater or less pressure will be exerted upon the liquid hydrocarbon, forcing it to enter the pores of the filaments and the molds, thus driving out the oxygen and replacing it with hydrocarbon. After this treatment the molds, with the filaments carried thereby, are placed in a suitable crucible of fire-clay, nickel, or other suitable material, as shown in Fig. 2 at D. The molds are covered and surrounded by powdered carbon and the crucible is tightly closed at the top by a cover, d', cemented or tightly closed and sealed in any other convenient manner. A tube, d, leads to a condenser, E, of any suitable character for receiving the vapors which come from the hydrocarbon with

which the filaments and molds have been saturated, and which arise from filaments themselves when the crucible D is subjected to heat sufficient to carbonize the filaments.

5 I claim as my invention—

The hereinbefore-described process of preparing filaments for incandescent electric lamps, which consists in winding the filaments upon carbon blocks, displacing the occluded

10 gases in the blocks and filaments, filling the

pores of the blocks and filaments with an inert fluid, and carbonizing the filaments.

In testimony whereof I have hereunto subscribed my name this 24th day of March, A. D. 1887.

EDWARD P. THOMPSON.

Witnesses:

DANL. W. EDGECOMB,  
CHARLES A. TERRY.